

Oct. 27, 1953

J. R. ERICKSON

2,656,654

GRINDING WHEEL

Filed Jan. 6, 1950

2 Sheets-Sheet 1



FIG. 1



FIG. 2



FIG. 3

By JOHN R. ERICKSON  
George G. Thompson  
Attorney

Oct. 27, 1953

J. R. ERICKSON  
GRINDING WHEEL

2,656,654

Filed Jan. 6, 1950

2 Sheets-Sheet 2

FIG. 4



FIG. 5



FIG. 6



Inventor

JOHN R. ERICKSON

By *George L. Compton Jr.*  
Attorney

## UNITED STATES PATENT OFFICE

2,656,654

## GRINDING WHEEL

John R. Erickson, Worcester, Mass., assignor to  
 Norton Company, Worcester, Mass., a corpora-  
 tion of Massachusetts

Application January 6, 1950, Serial No. 137,245

4 Claims. (Cl. 51—195)

1

The invention relates to grinding wheels. One object of the invention is to provide a rugged grinding wheel of unbrittle characteristics which can be dropped on the floor (even a concrete floor) and stepped upon without even cracking, the wheel being more or less relatively thin. Another object of the invention is to provide such a grinding wheel which will not fly apart even if it is cracked by some extraordinary abuse. Another object of the invention is to provide a rugged grinding wheel which is free cutting.

Another object of the invention is to provide a grinding wheel particularly suitable for use in smoothening the welds on automobile bodies which are formed when sections of steel plate are welded together and to provide a wheel particularly suitable for use in smoothening the welds on other fabricated metal or in smoothening protuberances, irregularities or rough spots of other kinds. Another object is to provide a grinding wheel which will take the place of coated abrasive discs (discs made out of heavy sand paper or heavy abrasive cloth) thus eliminating the frequent replacement of the abrading element, since grinding wheels made in accordance with this invention will outlast many such coated abrasive discs. Another object is to provide a grinding wheel having all the advantages of coated abrasive discs but without the disadvantages thereof especially the disadvantage of quick exhaustion of useful life. Another object is to provide a tool which will quickly take on a bevel or mitre on the periphery, since grinding wheels so shaped are exceedingly efficient for the purposes above indicated. Another object is to provide a wheel which can be used for the above purposes and also as a cutting-off wheel, for example to cut off gates and risers of castings. Another object is to provide a wheel suitable for removing rust and scale from steel plate.

Other objects will be in part obvious or in part pointed out hereinafter.

In the accompanying drawings illustrating a preferred procedure for manufacturing a wheel according to the invention and the wheel so produced together with a representation of the power tool upon which it may be used.

Figure 1 is an exploded view illustrating in section the several components of the wheel in the raw state.

Figure 2 is a cross sectional view of a mold partly filled, that is containing some of the components of Figure 1.

Figure 3 is a cross sectional view of the mold of Figure 2 completely filled and closed, that is the components having been pressed to unite to form the wheel.

Figure 4 is a plan view of the completed wheel.

2

Figure 5 is a cross sectional view of the wheel after it has acquired a bevel or mitre together with the mounting disc therefor.

Figure 6 is a perspective view of a power hand tool such as used for smoothening welds, etc. having the wheel of the invention secured thereon.

Referring first to Figure 1, I provide a quantity of dry granular mix 10 having organic bond. This comprises abrasive grains each granule of which is coated with the organic bond. As a practical matter the abrasive grains will usually be either aluminum oxide grains or silicon carbide grains. However other abrasives such as garnet or even diamonds can be used. Aluminum oxide abrasive is available in several different grades including the so-called regular grade which is a brown abrasive about 95%  $Al_2O_3$ , the white porous variety which is about 98% pure or better and contains a small percentage of soda, and recently developed aluminum oxide abrasive produced in discrete crystals and being usually better than 99%  $Al_2O_3$ . Silicon carbide abrasive is also available in several different grades such as the black grades and the green, the latter being the purest grade. All this is known to the art and any variety of these or other abrasives can be used.

While so far as the broad aspects of the invention are concerned many different organic bonds might be used I prefer to use available commercial grades of phenol formaldehyde resin otherwise known as resinoid. Unconverted phenol formaldehyde resin is available to the manufacturer in two forms, the solid phase material and the liquid phase material. For the production of a dry granular mix in which each abrasive granule is coated with an organic bond, the abrasive is placed in a mixing pan and then wet with a liquid and then, while continuing the mixing, bond in powdered form is added and eventually the abrasive coated with liquid picks up the powdered bond until each granule has an envelope of bond and the entire mix appears to be fairly dry even though it does contain liquid phase material. Thus the abrasive grains can be wet with liquid phenol formaldehyde resin and then solid phase powdered phenol formaldehyde resin can be added to complete the formation of the dry granular mix. On the other hand the abrasive grains can be wet with furfural and then powdered resin added. The powdered phenol formaldehyde resin available and which is hereinafter identified contains a minor percentage of creosol formaldehyde.

In describing an illustrative embodiment of the manufacture of a wheel according to the invention, I shall describe the manufacture of a wheel seven inches in diameter, one-eighth inch

thick and with a seven-eighths inch hole, the wheel having an off-set hub.

For the manufacture of this wheel a dry granular mix can be made from the following ingredients:

EXAMPLE I

*Dry granular mix ingredients*

|                                                          |      |
|----------------------------------------------------------|------|
| No. 24 grit size aluminum oxide abrasive,                |      |
| regular grade                                            | 4.74 |
| Powdered reactive phenol formaldehyde resin brand BR2417 | 1.67 |
| Carbon black                                             | .027 |
| Natural cryolite powder                                  | .68  |
| Furfural                                                 | 20   |
| Anthracene fractions from coal tar                       | 20   |

In making the mix the abrasive is placed in a mixing pan and mixing is started whereupon the furfural is slowly added. When all of the abrasive is wet, a mixture of the cryolite and the powdered phenol formaldehyde is added and mixing is continued until the powder is well distributed. Then the anthracene oil is added. This has the function of laying the dust. The cryolite improves the grinding action of the wheel, makes it stronger and also improves the consistency of the mix. With this small amount of furfural in the mix about 80% of the bond is loose in the mix. The carbon black gives a uniform color, to wit, black.

Referring now to Figures 2 and 3, I provide a steel mold consisting of a cylindrical mold band 11, a bottom plate 12, a top plate 13, and an arbor 14. For the manufacture of a wheel with an offset center, the bottom plate 12 and the top plate 13 can be shaped as shown. Further description of the mold would seem to be superfluous since the drawings are clear and molds of this general character are well known to everybody concerned with the manufacture of grinding wheels.

Figure 2 shows the mold with the mold band 11, the bottom plate 12 and the arbor 14, the top plate 13 being absent. The mold in this condition is filled with the various ingredients to be pressed as follows:

First a layer 15 of powdered resinoid is charged into the mold and levelled as shown. For a wheel seven inches in diameter, one-eighth inch thick and having a seven-eighths inch central hole the amount of material for the layer 15 should be about 10 grams. For this material I now prefer a phenol formaldehyde powder containing a minor percentage of polyvinyl butyral. This material is procurable on the market under the brand designation No. 795. With this material I mix about 1% by weight of carbon black. This phenol formaldehyde - polyvinyl - butyral combination cures quickly, makes a tough resinoid which has lower heat resistant properties than ordinary phenol formaldehyde resin. The purpose of this layer 15 is to form a protective coating for the nylon and also to prevent the cured wheel from sticking to the bottom mold plate 12. It is advantageous to have this layer heat sensitive because we want it to wear away readily during grinding.

I next place in the mold a 2-ply layer 16 of nylon leno cloth cut in the shape of a disc with a central hole. Nylon is, of course, the condensation product of hexamethylene diamine and adipic acid, while woven and knitted materials of nylon are known to everybody. The leno weave is the weave that has been known for generations for the manufacture of bolting cloth

as well as the so-called marquisette fabric. In leno weaving the warp threads are drawn in double and the harness frames instead of raising one section of the warp and lowering another section thereof move one of each pair of warp ends over and across the other thereof at each pick. All of this is well known in the weaving art. I have found that nylon leno cloth having twenty-one picks to the inch and twenty-one double sley is satisfactory. The weight of this material in a single ply is 3.6 ounces to the square yard. Furthermore this 2-ply nylon leno cloth was coated with a rubber compound of the following composition:

EXAMPLE II

*Composition of rubber coating on nylon leno cloth*

|                                     | Parts by weight |
|-------------------------------------|-----------------|
| Butadiene acrylic nitrile copolymer | 100             |
| Zinc oxide                          | 200             |
| Sulphur                             | 2               |
| Paracumarone                        | 50              |
| Carbon black                        | 3               |

The above ingredients are first thoroughly mixed (only the paracumarone is a liquid) then calendered into sheets and then dissolved in enough methyl ethyl ketone to make the material of the consistency of dough or slightly thinner. The nylon leno cloth is then run double between a pair of steel rolls and this dough-like material applied at the leading edge. The rolls are set together close enough to leave only a thin coating of the rubber compound. In the illustrative example of the invention the composition of Example II in the nylon leno cloth weighs 50% to 60% of the total of composition and cloth. After heating the cloth so treated to drive off the methyl ethyl ketone, it is cut into 2-ply discs 16 having a one inch central hole and being about six and seven-eighths inches in diameter. Making the 2-ply disc 16 slightly less in diameter than that of the final wheel eliminates a frayed edge in the finished product. The 2-ply disc 16 does not follow the depression 17 in the mold plate 12 because it is too stiff.

I next add a layer of 80 grams of the dry granular mix 10 which is levelled off in the mold. The mold is preferably on a revolving turn-table during filling which facilitates levelling.

I then place in the mold a single ply disc 18 of glass fabric. The glass fabric I have used had a plain weave with eighteen picks to the inch and eighteen sley and weighed 9.56 ounces per square yard. I prefer to use a single ply glass cloth disc only six and seven-eighths inches in diameter for the above stated reason of avoiding a frayed edge on the wheel and this disc may have a one inch central hole. This glass cloth as provided by the manufacturer has a coating of oily and starchy material thereon. I have found it advisable to heat the glass cloth at 300° C. for three hours which drives off the oils and chars the starch. This seems to stop the discs from fraying. It makes them stiffer and facilitates handling.

I next charge the mold with another layer of 80 grams of dry granular mix 10 and level it off. I then insert another single ply disc of glass cloth 18. I then add another layer of 10 grams of powdered resinoid 15 and level it off. I then insert the top plate 13 and the mold is now charged and ready for hot pressing. Prior to filling the mold it is advisable to coat all the

inside surfaces thereof with mineral oil which helps to keep the finished wheel from sticking to the mold.

I now take the filled mold to a hot press and press for fifteen minutes at a temperature of 160° C. at a pressure of 500 to 1000 pounds per square inch. After this the mold is removed from the press and allowed to cool and when it has cooled the mold is stripped and the wheel is removed. The pressure is not exactly critical although a fairly substantial pressure should be used, for example 500 pounds or more. If the mix is very flowable, a low degree of pressure should be used, otherwise resin will ooze out between the top plate and the mold band. In general I have found that the pressure should be not higher than 1500 pounds per square inch and not less than 300 pounds per square inch. In practice the movement of the top mold plate 13 is measured and when an average figure for the best wheels is found mold stops are set to close the mold to the stops regardless of slight variations in pressure involved in so doing. Molding to stops is now per se well known in the art.

The completed wheel 20 is shown in Figures 4, 5 and 6. It is a disc with an offset hub 21 and a central hole 22, a front face 23 and a rear face 24. After grinding the welds on automobile bodies, its periphery usually acquires a taper 25 but prior to grinding it has a square edge periphery 26. The front face 23 is desirably knurled and this way may be achieved as follows: the mold plate 13, being made of a soft steel such as cold rolled steel, is mounted in a lathe and then a knurling tool is fed against the inside face of the top plate 13 to make a ring of knurling and then the knurling tool is moved inwardly or outwardly and the operation is repeated until the flat portion 27 outward of the offset forming portion 28 has been knurled all over its surface. It is practically impossible to show this feature in Figure 2 but Figure 4 shows the knurling 30 thus illustrating the pattern on the top plate 13.

This knurling of the front face 23 gives the wheel a better appearance but additionally it improves its action when used as a cut-off wheel. For this reason the rear face 24 may also be knurled if desired. However up to now the rear face 24 has always been flat and the wheels have been found to be superior from all points of view.

The glass cloth discs 18 give strength to the wheel so that it is found it does not break until a speed of 30,000 surface feet per minute is reached. It is well known that grinding wheels of a given composition break at a given speed measured in surface feet per minute regardless of varying diameter provided the central hole is proportionately the same size in the different wheels, so therefore a breaking speed of so many surface feet per minute has a real meaning even though the diameter is not specified and the variation due to different ratios of the diameter of the central hole is usually a small variation. The nylon leno disc on the other hand keeps the wheel from flying to pieces after it has been cracked as by a severe blow. In other words, there is a cooperation between the two reinforcements in that one (the glass cloth) acts as a primary strengthener and the other acts as a secondary strengthener. Breakage of the glass cloth occurs before the nylon leno cloth breaks due to the greater stretchability of the nylon leno. Yet nylon is exceedingly strong and therefore al-

though a cracked wheel may not be as useful for grinding as an uncracked wheel, nevertheless the fact that it will not fly to pieces is vitally important because a hand tool that flies to pieces usually injures the operator. Wheels according to my invention are recommended for operation up to 11,000 surface feet per minute thus leaving a large factor of safety for protection of operators. At speeds of 11,000 surface feet per minute and below these wheels are highly efficient grinding wheels for the purposes indicated.

The purpose of the layer of resinoid 15 at the front face 23 is, besides preventing the cured wheel from sticking to the top plate 13, to prevent the knurling plate from injuring the woven glass disc 18. Thus this layer has a double function. The purpose of the layer 15 on the rear face 24 is not only to prevent sticking to the bottom mold plate 12 but also to improve the appearance of the wheel and furthermore I have found that both of these layers function to make the wheels stronger. I made up some wheels without layers 15 on the front face 23 and they were not so strong as those having the layers 15. Hence the provision of non-abrasive outside resinoid layers has several functions and generally stated results in a stronger and more durable wheel while at the same time it is found that it does not interfere with the grinding action. Still another reason for the provision of the layer 15 outside of the nylon disc 16 is that when the wheel is used as a cutting-off wheel the resinoid keeps the metal from cutting the nylon disc.

It has already been pointed out that the 2-ply disc 16 does not follow the depression 16 but rather lies flat in the mold. By reason of the heating of the glass cloth the discs 18 also lie flat in the mold. Thus after the disc 16 is laid down the mold being filled is a flat mold and this permits filling to achieve uniform density throughout the wheel. An air space 31 is left in the mold but as soon as the top plate 13 is pressed downwardly, the air disappears, probably along the arbor 14. At all events by proceeding as described practically perfect wheels can be produced.

The formula given in Example I represents more bond by volume than in the average resinoid bonded grinding wheel. This factor together with the large amount of free bond in the mixture (free bond is bond not attached to an abrasive granule) gives a good flow of resinoid through the glass cloth and the rubber coated nylon cloth during curing. This makes the wheels very strong. A wheel made according to Example I has about 32% abrasive by volume, the balance being practically all bond including the cryolite filler and the glass and nylon cloth. However good wheels can be made according to this invention using between 25% to 40% abrasive by volume with a porosity from 0% to 10%. The above volume percentages of abrasive are calculated on those portions of the wheel which result from the curing of the layers 19 of dry granular mix.

Many variations can be made in manufacturing this grinding wheel. For example, the coating on the nylon leno cloth could be natural rubber instead of butadiene acrylic nitrile copolymer or other rubber substitutes such as butadiene styrene copolymer could be used and other natural products such as gutta-percha. Instead of dissolving the rubber or synthetic rubber, all of which can be described as elastomers, in 75 methylethyl ketone, other solvents can be used

7 and I have used acetone with good results. But so far as the broad features of the invention are concerned, the nylon leno might be altogether uncoated.

Referring now to Figure 6, a typical power driven hand tool 35 for using the wheel 20 is shown. There are many varieties of hand tools that can use the wheel of this invention, but to give a typical example of the use of the wheel I have provided a perspective view of a particular hand tool 35 which comprises a metal casing 36 containing a motor having a shaft which drives bevelled gearing in a casing 34 attached to the casing 36 and the bevelled gearing drives a spindle 37 which has a threaded end 38 receiving a nut 39 which holds the wheel 20 against a hub 40 integrally connected to a back plate 41. Power is supplied to the tool 35 by electric cables 42 and the operator holds the hand tool 35 by means of handles 43 and 44. By means of 20 this or any other kind of hand tool the wheel 20 can be used for any of the purposes hereinbefore given.

Since this wheel is usually used for off hand grinding, figures with respect to material removed and wheel wear are not available. Wheels for off hand grinding are judged by the opinion of operators who use them who give their opinion on the basis of the ease with which the wheel cuts, the convenience of using the wheel, the 30 amount of production work which can be done before the wheel has worn out, the facility of grinding with it and most of all its safety characteristics, because many operators have been injured by the use of hand grinders. Wheels 35 constructed according to the present invention have been found to be superior in actual practice when judged by the above criteria. Wheels according to the above invention have been successfully used for all of the purposes set forth 40 in the objects hereinbefore stated.

While I have described my invention as embodied in a grinding wheel bonded with matured phenol formaldehyde resinoid, it is clear that parallel discs of woven glass cloth and of nylon cloth, whether of the leno weave or otherwise, can be connected and embedded by organic bond other than phenol formaldehyde. For example I could use natural rubber, butadiene acrylic nitrile, butadiene styrene, aniline formaldehyde or 45 alkyd resin. The nylon cloth is preferably of an open weave, that is to say you can see right through it, and the leno weave is the best open weave, but a fabric will be open if the pick and sley and size of yarn are properly selected as is well known in the weaving art and therefore 50 other open weaves may be used although they do not hold their shape as well as the leno weave.

It will thus be seen that there has been provided by this invention a grinding wheel in accordance with which the various objects hereinabove set forth together with many thoroughly practical advantages are successfully achieved. As many embodiments can be made of the above 55 invention and as many changes might be made in the embodiment above set forth, it is to be understood that all matter hereinbefore set forth or shown in the accompanying drawings is to be interpreted as illustrative and not in a limiting sense.

I claim:

1. A grinding wheel comprising a disc with an offset hub and a central hole centrally located in the hub and in the disc, said disc being made of abrasive grains bonded with a matured phenol-

8 formaldehyde resinoid, and said disc containing at least one reinforcement of woven glass cloth and containing at least one reinforcement of nylon leno cloth, the glass cloth and the nylon leno cloth extending from the hub to close to the periphery of the disc and the nylon leno cloth being closely adjacent to that side of the disc towards which the hub is offset.

2. A grinding wheel comprising a disc with an offset hub and a central hole centrally located in the hub and in the disc, said disc being made of abrasive grains bonded with a matured organic bond selected from the group consisting of phenol formaldehyde, natural rubber, butadiene acrylic nitrile, butadiene styrene, aniline formaldehyde, and alkyd resin, and said disc containing at least one reinforcement of woven glass cloth and containing at least one reinforcement of nylon leno cloth, the glass cloth and the nylon leno cloth extending from the hub to close to the periphery of the disc and the nylon leno cloth being closely adjacent to that side of the disc towards which the hub is offset.

3. A grinding wheel comprising a disc with a hole centrally located therein, said disc being made of abrasive grains bonded with a matured phenol-formaldehyde resinoid, and said disc containing at least one reinforcement of woven glass cloth and containing at least one reinforcement of nylon leno cloth, the glass cloth and the nylon leno cloth extending from near the hole to close to the periphery of the disc and the nylon leno cloth being closely adjacent to one side of the disc, the side opposite the side to which the nylon leno cloth is adjacent being the grinding side of the disc, whereby the nylon leno cloth which does not readily disintegrate will not impede the grinding operation or cause gumming of the grinding side.

4. A grinding wheel comprising a disc with a hole centrally located therein, said disc being made of abrasive grains bonded with a matured organic bond selected from the group consisting of phenol-formaldehyde, natural rubber, butadiene acrylic nitrile, butadiene styrene, aniline formaldehyde and alkyd resin, and said disc containing at least one reinforcement of woven glass cloth and containing at least one reinforcement of nylon leno cloth, the glass cloth and the nylon leno cloth extending from the hub to close to the periphery of the disc and the nylon leno cloth being closely adjacent to one side of the disc, the side opposite the side to which the nylon leno cloth is adjacent being the grinding side of the disc, whereby the nylon leno cloth which does not readily disintegrate will not impede the grinding operation or cause gumming of the grinding side.

JOHN R. ERICKSON.

References Cited in the file of this patent

UNITED STATES PATENTS

| Number    | Name           | Date           |
|-----------|----------------|----------------|
| 201,778   | Hart           | Mar. 26, 1878  |
| 1,010,040 | Gardner et al. | Nov. 28, 1911  |
| 1,686,938 | Stratford      | Oct. 9, 1928   |
| 1,884,436 | Weil           | Oct. 25, 1932  |
| 2,073,739 | Flatow et al.  | Mar. 16, 1937  |
| 2,085,211 | Budds et al.   | June 29, 1937  |
| 2,092,591 | Sohlstrom      | Sept. 7, 1937  |
| 2,094,556 | Anderson       | Sept. 28, 1937 |
| 2,138,882 | Robie          | Dec. 6, 1938   |
| 2,328,998 | Radford        | Sept. 7, 1943  |
| 2,475,517 | Ries et al.    | July 5, 1949   |